

2,859,167

## PRODUCTION OF BLOWN ASPHALTS IN THE PRESENCE OF A PHOSPHOROUS CONTAINING CATALYST

Joseph W. Van Wyk, Chicago, Ill., assignor to Standard Oil Company, Chicago, Ill., a corporation of Indiana

No Drawing. Application February 8, 1954  
Serial No. 409,008

13 Claims. (Cl. 208—5)

The present invention relates to an improved method of oxidizing certain high boiling hydrocarbon fractions to produce ductile, homogeneous asphalts of high solubility in carbon tetrachloride and low temperature susceptibility. In particular, the invention relates to an improved catalytic oxidation process, employing phosphorus compounds, e. g.  $P_2O_5$ , as catalysts for the transformation of high boiling petroleum residua and the like to asphaltic products.

The production of so-called "blown asphalts" by the air oxidation of various residual oils derived from petroleum is a well-known technique. Such "blown" asphalts are generally preferred for such purposes as coating irrigation canals, waterproofing conduits, roofing, etc. Many techniques have been proposed for the air oxidation of petroleum residua and one of the better processes embodies the use of a phosphorus catalyst such as  $P_2O_5$ . A process of this type is described and claimed in U. S. Patent No. 2,450,756 to Hoiberg. In that patent, a petroleum residuum is heated to a temperature in the range of from about 200° to about 350° F. and a small portion of that residuum is separately mixed with  $P_2O_5$  to form a catalyst slurry. The slurry is then introduced to the main body of the residuum and the total mix is heated to a temperature in the range of from about 400° to about 550° F. while vigorously agitating and introducing large quantities of air. Asphalts produced by this blowing technique have, generally speaking, excellent properties; but it has been found that certain requirements laid down by purchasers of such materials cannot be met consistently when applying this technique to the diverse types of residual oils which are available at refineries in different parts of the country. It has been found, however, that certain modifications in the process of the aforementioned patent result in unexpected improvements in the properties of blown asphalts so prepared, almost without regard to the source of high boiling hydrocarbon charge stock.

In accordance with the present invention, a suitable heavy petroleum fraction, of the type hereinafter described in detail, is heated to a temperature of at least 400° F. and preferably from about 460° to about 500° F. While this oil, e. g. a residuum, is being heated to such temperature, a relatively smaller amount of, for example, the same residual oil, is admixed with a stable phosphorus-containing catalyst at a temperature high enough to assure a fluid, readily pumpable slurry. The catalyst slurry thus produced is rendered smooth and homogeneous by vigorous agitation at such temperature. The time required for such homogenization will vary, of course, depending upon quantities of oil, type of oil, method of agitation, etc., but for most purposes from about 10 minutes to about 60 minutes and preferably at least about 20 minutes of mixing are adequate. At about the same time that the slurry preparation is begun or somewhat prior thereto, the main bulk of the residual oil to be oxidized is raised to oxidation temperature, i. e. about 460° F. and contacted with substantial quantities

of air. This thermal oxidation is carried out, in accordance with the present invention, for a period of at least one-half hour and preferably from about 2 to 4 hours before the catalyst slurry is introduced. Such thermal oxidation is generally continued until an increase in softening point of the residuum occurs equal to at least about 10° F. and preferably somewhat higher. Thus, for example, beginning the oxidation with a residuum having a softening point of 70° F., the thermal oxidation is continued until at least a softening point of 80°, and preferably from about 85° to about 95° F., is attained. Subsequent to such an increase in softening point, the catalyst slurry may be introduced into the residual oil rapidly, i. e. five minutes or less. The introduction of the catalyst slurry may, however, take substantially longer if desired. Thus, it may be carried out over a period of an hour or even longer. It has not been found necessary to so operate, however, and from a practical standpoint, it is desirable to complete the catalyst introduction in as short a period of time as possible.

One of the most difficult requirements to meet in the specifications of many blown asphalt purchasers is that the asphalt should have a solubility in carbon tetrachloride of at least 97%. Prior to the discovery of the present oxidation process, it has been very difficult to consistently produce asphalts having a high solubility. As a result of the present process, however, solubilities in excess of 99% are readily and consistently obtainable and from a variety of base oils. A typical specification for blown asphalt is that of the U. S. Bureau of Reclamation for "Catalytically Blown Asphalt Cement for Buried Asphalt Canal Lining" (ASTM D-165-42). The requirement of at least 97% solubility in  $CCl_4$  is a part thereof.

Whereas,  $P_2O_5$  is the preferred phosphorus-containing catalyst for use in accordance herewith, it should be understood that other stable phosphorus-containing materials may be used, e. g. red phosphorus or the stable sulfides of phosphorus, such as phosphorus pentasulfide, phosphorus sesquisulfide, phosphorus sulfide, etc.

It has been found that unless each of the above features of the present process are carefully adhered to, the consistent production of a high grade blown asphalt cannot be attained. Thus, for example, it is essential that the main body of residual oil be brought to oxidation temperature before any catalyst is introduced thereto, and it is also essential that at least about  $\frac{1}{2}$  hour of thermal oxidation of the stock take place before catalyst addition occurs. As indicated above, the preferred oxidation temperature is about 460° F. and unless the main body of the oil is at essentially this temperature during the so-called thermal oxidation period, the advantages inherent in this novel process are not fully realized. Thus, whereas the introduction of air during the preliminary stage may begin before the temperature is raised to about 460° F., the full effectiveness of the air treatment is not realized until the oil is substantially at the higher temperature. In any event, if air introduction is begun prior to attainment of temperature of about 460° F., it is necessary that air introduction continue for at least a half-hour after that temperature has been reached.

In accordance with the preferred method of introducing the catalyst slurry, the same is spread by means of a suitable spray nozzle over as much a surface of the residual oil as possible so that rapid and complete contact of catalyst and oil can be obtained substantially at once throughout a large volume of the oil. While not absolutely essential, it is highly desirable and in accordance with the preferred method of operation that the catalyst slurry be heated to a temperature between about 250° and 350° F. during the formation and preparation thereof. A rather high introduction temperature of this order

is indicated in any event because of the need for a fluid readily flowable slurry. This feature, while important, can be varied to some extent without unduly affecting the results of the process. The critical features of having the oil at oxidation temperature prior to catalyst addition and preliminary thermal oxidation for a period of at least one-half hour, cannot be varied beyond the rather narrow limits stated.

The customary residual oil employed in the production of blown asphalts for use in the present process is a crude oil residue derived from an asphaltic or semi-asphaltic base stock. Some so-called paraffinic base stocks of the non-asphaltic base class may be blown with air in accordance with the present invention to produce highly useful asphalts, however. It is preferred to employ heavy hydrocarbon fractions derived from such petroleums as those occurring in the U. S. Gulf Coast field, the so-called Mid-Continent crude residual oil and various other asphaltic petroleums. Consistent production of satisfactory blown asphalts has heretofore been unobtainable from residual oils derived from certain sour crudes of the type found in Wyoming. However, such oils have been readily oxidized to useful asphalts in accordance herewith. In addition to those residual oils commercially employed as asphalt base materials, lubricating oil distillates and solvent extracts resulting from the treatment of various petroleum fractions with such selected solvents as phenol, nitrobenzene, B,B'dichloroethylether (Chlorex),  $\text{SO}_2$ , etc., either alone or in combination with other high molecular weight petroleum fractions such as the residual oils or lubricating distillates, may be oxidized in accordance herewith to produce asphaltic products suitable for a wide range of uses. And whereas the present invention is particularly adapted to the production of waterproofing asphalts and the like, it should be apparent that a wide range of stocks may be handled to produce a variety of asphalt products.

For purposes of illustrating the oxidation of a typical Wyoming sour crude residual oil to produce an excellent canal lining asphalt, the following example is set forth:

#### EXAMPLE

114 tons of a Wyoming crude residual oil resulting from the atmospheric and vacuum reduction of a sour 45 Wyoming crude mixture was charged to a horizontal steel tank 14 feet in diameter by 14 feet long. Softening point of the starting material was  $69^\circ \text{ F}$ . and its SSF viscosity at  $180^\circ \text{ F}$ . was 220 seconds. The main body of the oil was raised to a temperature of  $460^\circ \text{ F}$ . and air was introduced at the rate of 40,000 cubic feet per hour and the oil was vigorously agitated. The initial air introduction was continued for about  $3\frac{1}{2}$  hours at the end of which time the softening point of the material in the tank had risen to  $84^\circ \text{ F}$ . During the preliminary thermal 50

5 oxidation of the main body in the oil, about 4 tons of the same stock was charged to a steam jacketed slurry tank equipped with a mixing impeller, gear pump, and circulating lines and the same was heated to a temperature of about  $325^\circ \text{ F}$ . After such temperature was attained, powdered  $\text{P}_2\text{O}_5$  in an amount sufficient to give an ultimate catalyst concentration in the main charge of about 1.2% was then vigorously admixed with the oil. Due to the small size of the steam jacketed slurry tank, it was necessary to prepare two separate slurry charges, in the first of which the catalyst comprises 20% by weight and in the second about 15% by weight. These slurries were then introduced to the main body of the oil in a period of about one hour (much less time would have been required if a single batch of slurry were available), all the while continuing the introduction of air at the rate of about 20,000 cubic feet an hour. Mechanical agitation of the slurry and the overall mixture was continued during slurry addition. The inspections of the final product 20 were as follows:

|                                        |      |
|----------------------------------------|------|
| Softening point, $^\circ \text{ F}$    | 179  |
| Penetration at $77^\circ \text{ F}$    | 63   |
| Ductility at $77^\circ \text{ F}$      | 4.75 |
| Solubility in $\text{CCl}_4$ , percent | 99.3 |

In Table 1 are set forth data demonstrating the effect of failing to observe the critical features of the present process. Thus is shown the effect of failing to have the 30 main body of the residuum heated to oxidation temperature prior to the introduction of the catalyst slurry. On the other hand, data are provided which demonstrate the disadvantage of adding the catalyst slurry to the residuum which although heated to the oxidation temperature had not been previously air-blown for at least about a half hour. The interdependence of the requirements that the residual oil be brought to oxidation temperature before any catalyst addition occurs and that such oil be blown for a substantial period of time prior to adding the catalyst, while not entirely understood, is apparent. It is obvious from the data in Table 1 that they are mutually dependent and that unless each of these requirements are observed, the consistent production of satisfactory blown asphalt has been difficult if not impossible to attain. And, whereas, the solubility of carbon tetrachloride is particularly susceptible to change when these important factors are disregarded, this is not the only characteristic which fails to pass specification and other physical properties have been shown to be inferior when the present process is not employed. In addition, it has been found that for best results, the slurry should be spread or sprayed over as large an area of the residuum as possible. Such, however, is not essential to the process and highly satisfactory products have been obtained by merely introducing at once a complete slurry charge. For

Table 1

| Run Number                                               | 1       | 2       | 3     | 4     | 5    | 6       |
|----------------------------------------------------------|---------|---------|-------|-------|------|---------|
| Viscosity at $180^\circ \text{ F}$ . (SSF)               | 220     | 220     | 102   | 102   | 214  | 124     |
| Percent $\text{P}_2\text{O}_5$ in Total Batch            | 1.15    | 1.15    | 1     | 1     | 1.25 | 1.25    |
| Percent $\text{P}_2\text{O}_5$ in Slurry                 | 20      | 20      | 20    | 20    | 18.5 | 19.6    |
| Slurry Temperature, degrees                              | 300-350 | 300-350 | 350   | 350   | 200  | 225-250 |
| Duration of Thermal Oxid. (Minutes)                      | 75      | 60      | 0     | 305   | 2.3  | 2.5     |
| Air Rate (cc./min./gram)                                 | ca. 2.5 | ca. 2.5 | 1     | 1     | 2.5  | 2.5     |
| Still Temp. During Slurry Addition, <sup>1</sup> degrees | 460     | 460     | 500   | 500   | 460  | 225-250 |
| Oxidation Temperature, degrees                           | 460     | 460     | 500   | 500   | 460  | 460     |
| Total Length of Oxid. (Thermal and Catalytic) (Minutes)  | 325     | 365     | 1,300 | 1,250 | 420  | 420     |
| Inspections of Final Product:                            |         |         |       |       |      |         |
| Softening Point, $^\circ \text{ F}$                      | 183     | 186     | 182   | 193   | 184  | 178     |
| Penetration at $77^\circ \text{ F}$                      | 54      | 50      | 58    | 71    | 64   | 62      |
| Ductility at $77^\circ \text{ F}$                        | 3.5     | 3.7     | 2.9   | 3.0   | 3.85 | 3.85    |
| Solubility in $\text{CCl}_4$ , percent                   | 99.65   | 99.78   | 95.2  | 98.1  | 89.1 | 92.1    |

<sup>1</sup> Slurry added rapidly—i. e. <1 minute.

<sup>2</sup> Air was turned on a short time before slurry was introduced, insignificant length of time.

comparative purposes a typical specification, viz. that of the U. S. Bureau of Reclamation, is set forth below:

|                                      |         |
|--------------------------------------|---------|
| Softening point, ° F.....            | 175-200 |
| Penetration at 77° F.....            | 50-60   |
| Penetration at 32° F.....            | NLT 30  |
| Penetration at 115° F.....           | NMT 120 |
| Ductility at 77° F.....              | NLT 3.5 |
| Solubility in CCl <sub>4</sub> ..... | NLT 97  |

The amount of catalyst employed in the oxidation of heavy oils to blown asphalts in accordance herewith should generally fall within the range of from about 0.1 to about 5.0 and preferably from about .75 to about 1.5% by weight of the total hydrocarbon charge. The slurry which is preferably formed from a portion of the main body of the residuum oxidized generally should comprise about 10 to about 25% catalyst and preferably from about 15 to about 20%. In any event, the slurry should have sufficient oil to permit adequate dispersion of the catalyst therein and yet not have too great an amount so as to dilute the catalyst to less than about a 10% concentration.

Air is introduced rapidly and in large quantities to the main body of the charge during both the preliminary thermal oxidation as well as during the catalytic oxidation to both oxidize and agitate the same. Rates of air introduction of from about 6 to about 70 cubic feet of air per minute per ton and higher may be employed but it is generally found that an amount of air from about 6 to 25 cubic feet of air per minute per ton of charge gives excellent results in plant practice. The introduction of the oxidizing gas is continued until the desired softening point is obtained, i. e. at least about 175.

The product may, if desired, be blown with steam toward the end of the air blow to remove any objectionable odors from the oil. Since steaming has a slight adverse effect on the penetration-softening point relationship, it should be started before the product of desired softening point is obtained.

Percentages given herein and in the appended claims are by weight based upon the total hydrocarbon oil charge, unless otherwise specified.

In the appended claims, the phrase "high molecular weight petroleum hydrocarbons" is employed to designate the residual oils or base stocks which may be oxidized to a blown asphalt in accordance herewith. In connection with the use of such term, it will, of course, be understood that the heaviest of petroleum hydrocarbons are not high molecular weight in the sense that many polymers are high molecular weight, but with the possible exception of a paraffin wax, essentially any heavy petroleum oil or residuum of the type defined hereinabove may be employed.

The phrase "hydrocarbon slurry oil" is employed in the appended claims to designate the oil used in the catalyst slurry and may, as indicated above in accordance with the preferred embodiment of the present invention, comprise the same oil as that being oxidized. On the other hand, it may comprise a different petroleum oil. Thus, it has been found that particular advantage may be gained by employing a somewhat lower boiling stock than that being oxidized in those instances wherein a very heavy residuum is being blown so as to permit easy handling of the catalyst slurry at somewhat lower temperatures. In particular, it has been found that lubricating oil extracts such as phenol extracts or Chlorex extracts may be used to excellent advantage. Other petroleum fractions such as lubricating oil base stocks, etc. may likewise be used. Synthetic polymers, e. g. high molecular weight butylene polymers, etc. may likewise be used.

In those instances where a portion of the oil being blown is used as slurry oil and particularly when blowing a heavy residuum, it has been found especially desirable,

although not essential, to use a portion of the thermally oxidized material for this purpose. Thus, the portion used as slurry oil is not separated from the main body until after a substantial period of thermal oxidation has taken place. It has been found that the resulting slurry may be more readily homogenized and is of much smoother appearance. Because the blowing does increase viscosity of the stock, the slurry oil should usually be withdrawn in less than about 4 hours for this purpose.

Whereas the heavy residuum when employed as slurry oil must be heated to about 300° F. in order to obtain a fluid, pumpable slurry, the use of an extract, for example of an SAE 20 or SAE 40 lubricating oil stock, permits slurry handling at temperatures of from about 100° to about 150° F. Furthermore, although the reasons for same are not entirely understood, there appears to be some definite improvement in ductility of the finished blown asphalt when a more fluid, lower-boiling slurry oil is employed. It should be understood, however, that whereas the terminology employed in the appended claims might indicate that the "hydrocarbon slurry oil" and the "high molecular weight hydrocarbon" are different oils, such is not necessarily the case.

Having thus described our invention, what I claim as novel and desire to protect by Letters Patent, is as follows:

1. The method of catalytically oxidizing suitable high molecular weight hydrocarbons to produce blown asphalts, which method comprises contacting said high molecular weight petroleum hydrocarbons with substantial quantities of air at a temperature in the range of from about 400° to about 500° F. for a period of at least about one-half hour, subsequently introducing a fluid homogeneous slurry of a phosphorus-containing catalyst selected from the group consisting of phosphorus pentoxide, stable phosphorus sulfides and red phosphorus in a hydrocarbon slurry oil to said high molecular weight petroleum hydrocarbons while at such a temperature, the amount of said phosphorus-containing catalyst being from about 0.1 to about 5.0% based upon the total weight of high molecular weight petroleum hydrocarbons and hydrocarbon slurry oil present, and continuing the introduction of air to the resulting admixture of catalyst, hydrocarbon slurry oil and high molecular weight petroleum hydrocarbons.

2. The method of claim 1 wherein the phosphorus-containing catalyst is phosphorus pentoxide.

3. The method of claim 1 wherein the hydrocarbon slurry oil employed to slurry phosphorus-containing catalyst is a portion of the high molecular weight petroleum hydrocarbons which had been separated from the main body of such hydrocarbons and admixed with the phosphorus-containing catalyst.

4. The method of claim 1 wherein the phosphorus-containing catalyst is phosphorus pentoxide and the hydrocarbon slurry oil employed to slurry the phosphorus catalyst is a portion of the high molecular weight petroleum hydrocarbons which had been separated from the main body of such hydrocarbons and admixed with the phosphorus-containing catalyst.

5. The method of claim 1 wherein the hydrocarbon slurry oil employed to slurry phosphorus-containing catalyst is an extract resulting from the solvent extraction of a lubricating oil base stock.

6. The method of claim 1 wherein the phosphorus-containing catalyst is phosphorus pentoxide and the hydrocarbon slurry oil is an extract resulting from the solvent extraction of a lubricating oil base stock.

7. The method of catalytically oxidizing suitable high molecular weight hydrocarbons to produce blown asphalts, which method comprises contacting said high molecular weight petroleum hydrocarbons with substantial quantities of air at a temperature in the range of from about 400° to about 500° F. for a period of about 2 to about 4 hours, subsequently introducing a fluid homo-

geneous slurry of a phosphorus-containing catalyst selected from the group consisting of phosphorus pentoxide, stable phosphorus sulfides and red phosphorus in a hydrocarbon slurry oil to said high molecular weight petroleum hydrocarbons while at such a temperature, the amount of said phosphorus-containing catalyst being from about 0.1 to about 5.0% based upon the total weight of high molecular weight petroleum hydrocarbons and hydrocarbon slurry oil present, and continuing the introduction of air to the resulting admixture of catalyst, hydrocarbon slurry oil and high molecular weight petroleum hydrocarbons.

8. The method of claim 7 wherein the phosphorus-containing catalyst is phosphorus pentoxide.

9. The method of claim 7 wherein the hydrocarbon slurry oil employed to slurry phosphorus-containing catalyst is a portion of the high molecular weight petroleum hydrocarbons which had been separated from the main body of such hydrocarbons and admixed with the phosphorus-containing catalyst.

10. The method of claim 7 wherein the phosphorus-containing catalyst is phosphorus pentoxide and the hydrocarbon slurry oil employed to slurry the phosphorus catalyst is a portion of the high molecular weight petroleum hydrocarbons which had been separated from the main body of such hydrocarbons and admixed with the phosphorus-containing catalyst.

11. The method of claim 7 wherein the hydrocarbon slurry oil employed to slurry phosphorus-containing catalyst is an extract resulting from the solvent extraction of a lubricating oil base stock.

12. The method of claim 7 wherein the phosphorus-containing catalyst is phosphorus pentoxide and the hydrocarbon slurry oil is an extract resulting from the solvent extraction of a lubricating oil base stock.

13. The method of claim 7 wherein the hydrocarbon slurry oil employed to slurry the phosphorus-containing catalyst is a portion of the high molecular weight petroleum hydrocarbons which had been separated from the main body of such hydrocarbons after said main body of hydrocarbons had been subjected to a substantial period of thermal oxidation.

References Cited in the file of this patent

UNITED STATES PATENTS

|               |                   |               |
|---------------|-------------------|---------------|
| 20. 2,076,799 | Thurston          | Apr. 13, 1937 |
| 2,121,437     | McConnell         | June 21, 1938 |
| 2,179,208     | Burk et al.       | Nov. 7, 1939  |
| 2,179,988     | Whitacre          | Nov. 14, 1939 |
| 25. 2,415,697 | Knowles et al.    | Feb. 11, 1947 |
| 2,450,756     | Hoiberg           | Oct. 5, 1948  |
| 2,455,709     | Spelshouse et al. | Dec. 7, 1948  |
| 2,676,910     | Edson             | Apr. 27, 1954 |